

# UNITED STATES PATENT OFFICE.

AUGUSTUS ROSENBERG, OF LONDON, ENGLAND.

## METHOD OF AND MEANS FOR CLEANING THE SURFACES OF ARTICLES MADE OF SILVER AND OTHER METALS.

1,049,603.

Specification of Letters Patent.

Patented Jan. 7, 1913.

No Drawing.

Application filed August 28, 1912. Serial No. 717,482.

To all whom it may concern:

Be it known that I, AUGUSTUS ROSENBERG, a subject of the King of Great Britain, and resident of 259 High Holborn, London, 5 W. C., England, engineer, have invented a certain new and useful Method of and Means for Cleaning the Surfaces of Articles Made of Silver and other Metals, of which the following is a specification.

10 It has heretofore been proposed to clean silver articles by immersing them in a warm aqueous alkaline solution and bringing them into contact with a plate made of a metal electro-positive with respect to silver (e. g. 15 aluminium), the cleaning being effected by the nascent hydrogen generated which chemically reduces and removes the film of oxid, sulfid, or other reducible salt or salts present on the surface of the article. In practice, 20 this method of cleaning is unsatisfactory for the reason that the plate of electro-positive metal speedily becomes oxidized, thus preventing the alkaline reagent from attacking the metal plate. Moreover it is essential that 25 effective mechanical contact between the metal plate and the article to be cleaned should take place and this is impracticable when a number of articles are to be cleaned at the same time. Finally, the cleaning of 30 the surface is unequal and the bulk of the hydrogen generated is wasted.

The object of the present invention is to obviate these disadvantages.

According to my invention the electro-positive metal is in granular comminuted or pulverulent form so that it will become completely disseminated in the alkaline bath and remain in suspension therein for a certain time. Hence the surface of the electro-positive metal in contact with the solution is very considerable and is obviously greatly in excess of the surface exposed to the action of the alkaline solution when a plate of electro-positive metal of equal weight is employed. Furthermore, the sub-divided state of the metal, when it has been added to the alkaline solution, gives rise to numerous intense local chemical reactions which bring about the production of nascent hydrogen 50 wherever a particle of metal is in suspension in said solution. In operation, the article itself acts as cathode in the electrolyte constituted by the alkaline solution, and all the particles of the electro-positive metal constitute minute anodes which make innumer-

able contacts with the article to be cleaned and becoming gradually dissolved set up innumerable local electric circuits each of which possesses exceedingly low resistance owing to the small distance separating the 60 anode from the cathode of each individual circuit.

As electro-positive metal I prefer to employ aluminium as this metal is more active than others in an alkaline solution, but any other metal (e. g. magnesium, aluminium, zinc, tin, cadmium) electro-positive with respect to the surface to be cleaned, may be employed. I may employ as electro-positive metal either a mixture or an alloy of metals 70 (e. g. magnalium). When a mixture of electro-positive metals is used they may either be in their elementary i. e. unoxidized state, or the particles of one metal may be coated with a deposit of another metal to 75 form a plurality of galvanic couples. To illustrate what I mean I may instance galvanic couples constituted by particles of zinc coated with a spongy deposit of copper.

As the electro-positive metal (or mixture 80 of metals or alloy, or metal covered with a deposit of another metal to form a couple, as the case may be), is in the comminuted or pulverulent state, it can be intimately mixed with the alkaline reagent and the mixture 85 made up either as a powder or in block or paste form.

In order to prevent premature change in the chemical state of the electro-positive metal or to bind the mixture, the particles 90 of the ingredients forming the mixture may be coated with an inert substance such as paraffin, resin or the like or, when the mixture is to be made up into a paste, the ingredients may be mixed with an inert liquid 95 substance such as glycerin.

The relative proportions of the ingredients may obviously vary within wide limits, but I have found that, for cleaning silver for example and when aluminium is used as 100 electropositive metal, one part by weight of aluminium to 125 parts by weight of alkaline reagent will produce good results.

As alkaline reagents, alkaline salts (e. g. borax, sodium borate) sodium or potassium carbonate or caustic alkalis or alkaline earths mixed with salts such as bicarbonates, may be employed to form an alkaline solution.

Although I have only referred to the 110

cleaning of silver articles I would have it understood that my invention may be used for cleaning articles made of certain other metals. For example, the "tarnish" on articles made of nickel, tin and gold may be readily and effectually removed by immersing them in a bath constituted by a mixture of the above mentioned ingredients. The article to be cleaned is allowed to remain in the bath for a length of time depending on the amount of "tarnish" to be removed and after withdrawal, is rinsed in water and dried.

Claims.

15. 1. The method of cleaning the surface of a metal article which consists in immersing the article in an aqueous alkaline solution containing a metallic substance electro-positive in respect of the surface to be cleaned in granular or comminuted form.
20. 2. The method of cleaning the surface of a metal article which consists in immersing the article in an aqueous alkaline solution containing a plurality of metallic substances electro-positive in respect of the surface to be cleaned in granular or comminuted form.
25. 3. The method of cleaning the surface of a metal article which consists in immersing the article in an aqueous alkaline solution containing a metallic substance electro-positive in respect of the surface to be cleaned in granular or comminuted form, the individual particles of said metallic substance being coated with a deposit of another metal to form galvanic couples.
30. 4. As a new article of manufacture for cleaning the surface of a metal article, a mixture of granular or pulverulent materials including a metallic substance electro-positive in respect of the surface to be cleaned and an alkaline substance capable of forming in conjunction with water an aqueous electrolyte.
35. 5. As a new article of manufacture for cleaning the surface of a metal article, a mixture of granular or pulverulent materials including a plurality of metallic substances electro-positive in respect of the surface to be cleaned, and an alkaline substance capable of forming in conjunction with water an aqueous electrolyte.
40. 6. As a new article of manufacture for cleaning the surface of a metal article, a mixture of granular or pulverulent materials including a metallic substance electro-positive in respect of the surface to be cleaned and an alkaline substance capable of forming in conjunction with water an aqueous electrolyte, the individual particles
45. 7. As a new article of manufacture for cleaning the surface of a metal article, a mixture of granular or pulverulent materials including a metallic substance electro-positive in respect of the surface to be cleaned and an alkaline substance capable of forming in conjunction with water an aqueous electrolyte, and a deposit of another metal to form galvanic couples.
50. 8. As a new article of manufacture for cleaning the surface of a metal article, a mixture of granular or pulverulent materials including a metallic substance electro-positive in respect of the surface to be cleaned coated with an inert substance to prevent premature chemical change, and an aqueous electrolyte.

70. 9. As a new article of manufacture for cleaning the surface of a metal article, a mixture of granular or pulverulent materials including a plurality of metallic substances electro-positive in respect of the surface to be cleaned, the individual particles of said metallic substances being coated with an inert substance to prevent premature chemical change, and an alkaline substance capable of forming in conjunction with water an aqueous electrolyte.

75. 10. As a new article of manufacture for cleaning the surface of a metal article, a mixture of granular or pulverulent materials including a metallic substance electro-positive in respect of the surface to be cleaned, the individual particles of which metallic substance being coated with a deposit of another metal to form galvanic couples which themselves are coated with an inert substance to prevent chemical change, and an alkaline substance capable of forming in conjunction with water an aqueous electrolyte.

80. 11. As a new article of manufacture for cleaning the surface of a metal article, a mixture of granular or pulverulent materials including a metallic substance electro-positive in respect of the surface to be cleaned, the individual particles of which metallic substance being coated with a deposit of another metal to form galvanic couples which themselves are coated with an inert substance to prevent chemical change, and an alkaline substance capable of forming in conjunction with water an aqueous electrolyte.

85. 12. As a new article of manufacture for cleaning the surface of a metal article, a mixture of granular or pulverulent materials including a metallic substance electro-positive in respect of the surface to be cleaned, an alkaline substance capable of forming in conjunction with water an aqueous electrolyte, and an inert binding agent.

90. 13. As a new article of manufacture for cleaning the surface of a metal article, a mixture of granular or pulverulent materials including a plurality of metallic substances electro-positive in respect of the surface to be cleaned, an alkaline substance capable of forming in conjunction with water an aqueous electrolyte, and an inert binding agent.

95. 14. As a new article of manufacture for cleaning the surface of a metal article, a mixture of granular or pulverulent materials including a metallic substance electro-positive in respect of the surface to be cleaned whose individual particles are coated with a deposit of another metal to form galvanic couples, an alkaline substance capable of forming in conjunction with water an aqueous electrolyte, and an inert binding agent.

100. 15. As a new article of manufacture for cleaning the surface of a metal article, a mixture of granular or pulverulent materials including a metallic substance electro-positive in respect of the surface to be cleaned coated with an inert substance to prevent premature chemical change, and an aqueous electrolyte.

alkaline substance capable of forming in conjunction with water an aqueous electrolyte, and a binding agent.

14. As a new article of manufacture for cleaning the surface of a metal article, a mixture of granular or pulverulent materials including a plurality of metallic substances electro-positive in respect of the surface to be cleaned, the individual particles of which are coated with an inert solid substance to prevent premature chemical change, an alkaline substance capable of forming in conjunction with water an aqueous electrolyte and a binding agent.
15. As a new article of manufacture for
- cleaning the surface of a metal article, a mixture of granular or pulverulent materials including a single metal electro-positive in respect of the surface to be cleaned, the particles of which are coated with a deposit of another metal to form galvanic couples which themselves are coated with an inert substance to prevent chemical change, an alkaline substance capable of forming with water an aqueous electrolyte, and a binding agent.

AUGUSTUS ROSENBERG.

Witnesses:

H. D. JAMESON,  
O. J. WORTH.